

Feb. 25, 1958

A. J. HATHAWAY III

2,824,794

## PROCESS FOR FUSION OF HIGH-MELTING METALS

Filed May 18, 1954



INVENTOR.  
Augustus J. Nathaway, III  
BY  
Ashlan F. Harlan Jr.

**ATTORNEY**

1

2,824,794

## PROCESS FOR FUSION OF HIGH-MELTING METALS

Augustus J. Hathaway III, Niagara Falls, N. Y., assignor to National Lead Company, New York, N. Y., a corporation of New Jersey

Application May 18, 1954, Serial No. 430,615

4 Claims. (Cl. 75—84)

This invention relates to the melting or fusion of high-melting metals and is particularly concerned with the fusion of high-melting reactive metals such as titanium and zirconium and alloys of such metals.

Such metals are usually produced as a sponge or in powder form which must be fused either to form ingots, that may be converted by machining, rolling or other known processes into desired articles or shapes, or to form cast articles. Melting of these reactive metals is, however, not a simple procedure since at elevated temperatures they react with the oxygen and nitrogen of the air and melting must therefore be carried out in the absence of air. In addition, these reactive metals, when molten, tend to attack the refractory materials from which are formed the refractory containers in which the metal is fused or held in the fused state. Aside from the consequent damage to the containers, such attack results in contamination of the metal. With graphite containers an undesirably large pick-up of carbon is likely to occur. When oxide-type refractories are used, the reactive metal picks up not only metallic impurities but also, and more importantly, oxygen. It has been found that even quite small amounts of oxygen are deleterious as the hardness of the metal is greatly increased thereby. The consequent impairment of working properties, such as ductility and malleability, may be so great that working of the metal is difficult or impossible.

It is therefore an object of the present invention to provide a method for fusing high-melting metals and alloys in which contamination of the metal or alloy is minimized.

Another object of the invention is to provide a method for fusing high-melting metals and alloys which results in insignificant or relatively slight increase in hardness of the metal or alloy.

A further object of the invention is to provide a method for fusing high-melting metals and alloys which involves the use of a crucible that is capable of resisting attack by the molten metals and alloys.

Another object of the present invention is to provide a crucible suitable for fusing high-melting, reactive metals without significant increase in the hardness of said metals.

Other objects and advantages of the present invention will be apparent from the following description taken in conjunction with the accompanying drawings in which:

Figure 1 is a vertical sectional view through an enclosed furnace which may conveniently be employed in the fusion of high-melting metals and alloys in accordance with the present invention and the casting of ingots thereof;

Figure 2 is a vertical sectional view through a modified form of crucible adapted for carrying out the present invention; and

Figure 3 is a horizontal sectional view taken on the line 3—3 of Figure 2 of the modified crucible shown in Figure 2.

2

In copending application Serial No. 260,946, filed December 10, 1951, now Patent No. 2,678,887, issued May 18, 1954, of which the present application is in part a continuation, it is disclosed that refractories containing large amounts of calcium oxide and smaller amounts of both zirconium dioxide and titanium dioxide are highly resistant to hydration and may be satisfactorily used in the fusion of high melting reactive metals such as titanium, zirconium and alloys of these metals. In such use it has been found that the refractories are so resistant to attack by the molten metals that only a relatively slight or insignificant increase in hardness of the metal occurs.

As set forth in the above mentioned application, such refractories may be formed into crucibles or in other refractory shapes according to conventional or other known procedures. In many instances it will be found desirable to employ a prefired grog, which has been reduced to granular form, in forming crucibles for use in melting titanium, zirconium and the like. As is well known, the use of a prefired grog materially reduces shrinkage in the formed bodies and also reduces the tendency of the bodies to crack during firing. In making crucibles for carrying out the process of the present invention the grog employed may be of any desired composition and the desired final composition of the fired crucible can be obtained by mixing with the grog appropriate quantities of the various constituents. The grog may either be merely sintered or, if desired, may be actually fused prior to reduction to granular form.

As further pointed out in the copending application referred to, in preparing mixes from which crucibles suitable for carrying out the process of the present invention may be formed, it is possible to use either the metal oxides as such or substances which, when fired, are converted to the several oxides,  $\text{CaO}$ ,  $\text{ZrO}_2$  and  $\text{TiO}_2$ , which are desired in the final product. Thus, for example, calcium carbonate, calcium hydroxide or calcium nitrate might be used in the raw mix, since upon heating these materials are converted to calcium oxide. Similarly, for example, the  $\text{TiO}_2$  and  $\text{ZrO}_2$  may be provided by using rutile, titanium hydroxide or titanium sulfate for the former and baddeleyite, zirconium sulfate or hydrated zirconium oxide (zirconium hydroxide) for the latter. Calcium zirconate and/or calcium titanate may also be used as ingredients since each of these materials is a combination of two of the oxides desired in the mix.

In carrying out the invention of the present application the high-melting metal or alloy is placed in a container or crucible of a  $\text{CaO}-\text{ZrO}_2-\text{TiO}_2$  refractory and heated in an inert atmosphere to fuse the metal. The metal may then be permitted to solidify or freeze in the crucible, the ingot resulting being removed from the crucible when the latter has been cooled and taken from the furnace, or, alternatively, the molten metal may be poured into a mold. The fusion is preferably carried out in an inductively heated electric furnace which, of course, must be enclosed to prevent access of air to the molten metal. The furnace enclosure may be evacuated or an atmosphere of an inert gas such as argon or helium may be provided therein. In Figure 1 of the drawings there is shown an apparatus suitable for the fusion of metals such as titanium, zirconium or alloys thereof and casting of the fused metal or alloy into a mold, all either in vacuum or in an inert gas atmosphere.

In Figure 1 the numeral 11 indicates the crucible in which the desired metal or alloy is melted. Preferably, the crucible is round in cross section and comprises a cylindrical wall 12 and a bottom 13 of somewhat greater thickness than the wall. A pouring lip 14 is preferably provided on the periphery of the open end of the crucible. The crucible 11 is supported within the furnace enclosure 16 on a refractory plate 17 carried by a pedestal 18 and

is surrounded by a casing 19, the upper portion of which at least, is formed of electrically nonconductive, refractory material such, for example, as mica or asbestos. Within the casing 18, around the crucible 11, there is provided a mass 21 of granular refractory material which serves to protect the crucible from shock and as thermal insulation therefor. Between the casing 19 and the crucible 11 at the top of the mass 21, there is provided a refractory annulus 22 which prevents the granular refractory material from spilling when the furnace is tilted. Spirally wound around the casing 18 is an electrical conductor 23 the ends of which extend outwardly through the enclosure 16 and through the conduit 24 to make connections with a suitable source of electric power (not shown).

At its top, the enclosure 16 is provided with a large opening and a removable cover 28 therefor. Extending through a gland 32 in the cover 28 is a reciprocatable rod 33 to the lower end of which there is attached a refractory crucible cover 34. By lowering or raising the rod 33 the cover 34 may be placed on the crucible top or removed therefrom to permit inspection of the crucible contents through the sight glass 36 and pouring of the metal.

Attached to the side wall of the enclosure 16 is a tubular extension 38 within which there is positioned by clamps, wedges or similar suitable means (not shown) a mold 39. The outer end of the extension 38 is provided with a pivoted closure 41 which may be opened to permit removal of the mold. The enclosure 16 is provided with aligned, oppositely disposed trunnions 43 by which it is pivotally mounted. The trunnions are so located that when the enclosure is rotated in a clockwise direction, as viewed in Figure 1, the contents of the crucible 11 will pour into the mold 39. One of the trunnions 43, as shown, is tubular and the bore 44 thereof is connected to a vacuum pump (not shown) by means of which the interior of the enclosure 16 may be evacuated. There is also provided in the side wall of the enclosure a nipple 46 through which communication with the interior of the enclosure may be obtained.

In carrying out the process of the present invention in apparatus like that shown in Figure 1, the charge of high-melting metal or alloy is placed in the crucible 11 and a suitable mold is placed in the extension 38 in proper position to receive molten metal from the crucible. The extension 38 is thereafter sealed by the closure 41 and the cover 28 is secured on the enclosure 16 by suitable means (not shown). The enclosure is then evacuated through the bore 44. When the air has been removed from the enclosure the crucible contents may be heated by supplying high frequency electric current to the conductor coil 23. When the metal or alloy has melted the furnace is tilted and the molten metal pours into the mold 39. Melting of the metal is facilitated by the use of the crucible cover 34 which reflects heat back into the crucible.

After pouring the fused metal or alloy into the mold the furnace is allowed to cool. The mold may be removed when there is no longer danger of reaction between the metal ingot therein and the air. Instead of providing a vacuum in the enclosure 16 it may be desired to use an inert gas such as helium or argon. Such gas may be admitted through the nipple 46. In some cases, even when using an inert gas atmosphere it may further be desired to employ a slight sub-atmospheric pressure, obtained by use of a vacuum pump (not shown) connected to the bore 44, so that any fumes given off in the furnace will be drawn therefrom and view of the crucible through the sight glass 29 will not be obscured. If desired, of course, the fused metal or alloy may be permitted to solidify in the crucible instead of pouring it into a mold.

The fusion of titanium in crucibles formed from several compositions of the type described above is set forth in the following examples.

#### Example 1

A quantity of blocks of previously sintered titanium having an average Brinell hardness number of 352 were placed in a crucible having the composition  $\text{CaO}-90\%$ ,  $\text{ZrO}_2-7\%$ ,  $\text{TiO}_2-3\%$ . The crucible was then placed in an induction furnace in an evacuated chamber and the titanium was melted, remaining at least partially molten for 15 minutes. The metal was then allowed to cool in the crucible. When cool, the titanium was removed from the crucible, adherence to the crucible being slight. The latter was in good condition, showing little erosion and only moderate cracking. The Brinell hardness of the titanium ingot obtained was 388. By analysis, the ingot was found to have an oxygen content of less than .30%. Since the average oxygen content of the charged metal was .287% it is obvious that the oxygen pick-up was very small.

The crucible used in this example was formed by ramming a granular grog of appropriate composition, the grog having been previously mixed with a small amount of a solution of an organic binder for imparting green strength thereto, and after drying was fired to a maximum temperature of about 3350° F.

#### Example 2

A number of previously sintered titanium blocks having an average Brinell hardness of 352 were placed in a crucible having the composition  $\text{CaO}-85\%$ ,  $\text{ZrO}_2-10\%$ ,  $\text{TiO}_2-5\%$  and fused in an evacuated induction furnace. The metal was at least partially molten for 15 minutes and was completely molten for more than 3 minutes. The crucible was then cooled and the titanium ingot removed. No difficulty was experienced in such removal since the adherence of the metal to the crucible was low. Inspection of the crucible showed only slight erosion thereof. The ingot obtained had a Brinell hardness of 367 and an oxygen content of less than .30%.

The crucible employed in carrying out this fusion was cast from a deaired slip containing 856 parts by weight  $\text{CaCO}_3$ , 91 parts by weight  $\text{CaZrO}_3$ , and 53 parts by weight  $\text{CaTiO}_3$  suspended in 190 parts by weight of water containing 11 parts of sodium alkyl naphthalene sulfonate and 2 parts of octyl alcohol. It was then dried and fired to a maximum temperature of about 3080° F.

#### Example 3

A number of titanium blocks like the ones used in Examples 1 and 2 were placed in a crucible having the composition  $\text{CaO}-80\%$ ,  $\text{ZrO}_2-12\%$ ,  $\text{TiO}_2-8\%$ . The crucible containing the metal was then placed in an induction furnace and the metal was melted in vacuum. It was at least partially molten for 5 minutes and was wholly molten for 2 minutes. The metal was allowed to cool in the crucible and the resulting ingot was then readily removed. The interior of the crucible showed no material erosion. The titanium ingot had a Brinell hardness of 321 and an oxygen content by analysis of approximately .28%.

The crucible used in fusing the titanium in this example was formed by casting a deaired slip containing, by weight, 799 parts of  $\text{CaCO}_3$ , 114 parts  $\text{CaZrO}_3$ , and 87 parts of  $\text{CaTiO}_3$ , all in finely divided form, suspended in a mixture of 195 parts of water, 11 parts sodium alkyl naphthalene sulfonate and 2 parts of octyl alcohol. After drying it was fired to a maximum temperature of about 3050° F.

#### Example 4

A crucible having the composition  $\text{CaO}-39\%$ ,  $\text{ZrO}_2-37\%$ ,  $\text{TiO}_2-24\%$  was charged with a quantity of slightly compacted titanium powder, the metal having substantially the same composition and hardness as that in the blocks charged in Examples 1-3. The charged crucible was then placed in an induction furnace located in an evacuated enclosure and the titanium was melted. The metal was completely molten for 3 minutes and par-

tially molten for 6 minutes. After the crucible cooled it was taken from the furnace and the metal ingot was removed. The crucible was in good condition and the titanium ingot obtained was found to have a Brinell hardness of 363 and an oxygen content less than .30%.

The crucible used in carrying out the fusion of the example was formed by ramming a moistened grog of the desired composition in substantially the same manner as in Example 1 and was fired to a maximum temperature of about 3050° F.

As heretofore mentioned, the novel process of the present invention is also valuable for fusion of alloys of high-melting metals such as titanium, zirconium and the like. Such use is illustrated in the following examples.

*Example 5*

A quantity of a chrome-iron titanium alloy containing approximately 95.6% titanium was charged as scrap into a crucible having the composition  $\text{CaO}$ —80%,  $\text{ZrO}_2$ —12%,  $\text{TiO}_2$ —8%. The crucible was mounted in an induction furnace of the type shown in Figure 1. After first evacuating the system the scrap was melted while feeding argon into the enclosure and maintaining therein an absolute pressure of about 17 inches of mercury. When the charge was molten the furnace was tilted and the contents of the crucible were poured into a cast iron mold. The average Brinell hardness of the scrap charged was 325, while the average hardness of the ingot obtained in the mold was 331. The crucible showed no signs of erosion.

The crucible used in the foregoing example was formed by ramming a mixture of various sizes of particles of electrically fused grog of the composition mentioned above. Before ramming the grog was moistened with a small amount of a solution of an organic temporary binder. After ramming, the crucible was dried and then burned by firing it to a maximum temperature of about 3250° F.

*Example 6*

Using the same crucible that was used in Example 5 another charge of the chrome-iron titanium base alloy scrap was fused in substantially the same manner. The titanium alloy ingot from the mold had a Brinell hardness of 350 whereas the average Brinell hardness of the scrap charged was 345. The crucible after use was in excellent condition.

Including the melts of Examples 5 and 6, a total of 7 melts was successfully made in the same crucible and the crucible was still in good condition. This fact shows that attack of the crucible by the molten metal is minimized.

It will be evident from the preceding examples that titanium and titanium alloys may be fused in crucibles, having compositions of the character described and claimed in the copending application above referred to, with only relatively small, and in some cases negligible, increases in hardness. Comparable results may be obtained in the fusion of zirconium, hafnium, and other high-melting reactive metals, and alloys thereof.

As explained above, in carrying out the novel process of the present invention the fused high-melting metal may, if desired, be allowed to solidify in the container or crucible in which it is fused. Thus, the crucible serves as a mold for the metal. It will be obvious, therefore, that if a separate mold is employed into which the molten metal is poured, the mold may be formed of a



refractory of the type with which the present application is concerned. Either ingots or castings of various desired shapes may be thus formed.

In the foregoing description and discussion reference has been made to crucibles, molds, and other refractory bodies formed entirely from a  $\text{CaO-ZrO}_2-\text{TiO}_2$  mix. It will be understood, however, that there may also be used refractory bodies having composite structures. In such bodies the portions in which the molten, reactive,

high-melting metal or alloy is held may be formed of such  $\text{CaO-ZrO}_2-\text{TiO}_2$  compositions while the rest of the bodies may be formed of other suitable refractory materials.

5 A crucible of the last mentioned type is shown in Figures 2 and 3 of the accompanying drawings. The crucible 51 comprises an inner, cup-like, container portion 52 having an outwardly projecting annular rim 53 around its open upper end and a concentric, outer, cup-like portion 56 in contact with the inner portion 52. The latter may be formed of a  $\text{CaO-ZrO}_2-\text{TiO}_2$  refractory such, for example, as any one of the compositions mentioned in Examples 1-4. The outer portion 56 may be formed of any other refractory which is serviceable at the desired temperature of use since, even though it would be readily attacked by the molten metal, it does not come into contact therewith. Among the refractory materials suitable for forming the outer portion 56 are magnesia and zirconia.

10 Composite crucibles of the type just described may be produced in any suitable and convenient manner. Thus, for example, one or the other of the two portions may be first formed and the other portion then rammed or cast thereon. When only a relatively thin metal-resistant portion or lining is desired, the interior of a crucible of other refractory material may be sprayed, painted, troweled or the like with a slurry or paste of a suitable  $\text{CaO-ZrO}_2-\text{TiO}_2$  mix. In some cases the outer portion may be formed of refractory blocks or shapes cemented together

15 by a suitable cement.

20 It will be understood that the raw materials used in forming crucibles or other containers, such as molds, for use in carrying out the process of this invention need not be chemically pure since minor amounts of normal impurities may be tolerated in such bodies. Indeed, as pointed out in the copending application referred to above, dolomite, which contains substantial amounts of magnesium carbonate along with calcium carbonate, may be used instead of ordinary calcium carbonate as a source of  $\text{CaO}$ .

25 In general, crucibles or other containers suitable for carrying out the present invention may have such compositions that the constituent oxides,  $\text{CaO}$ ,  $\text{ZrO}_2$  and  $\text{TiO}_2$ , exclusive of impurities, fall within the following ranges of proportions,  $\text{CaO}$ —90% to 39%,  $\text{ZrO}_2$  7% to 37%, and  $\text{TiO}_2$ —3% to 24%.

30 In the foregoing description and the following claims percentages are, unless otherwise indicated, percentages by weight. Further, the term "inert atmosphere" is intended to include a substantial vacuum as well as an atmosphere of inert gas and the term metal, except where a contrary intention is evident, is meant to include alloys.

I claim:

35 1. A process for fusing high-melting reactive metals of the class consisting of titanium and titanium-base alloys without significantly increasing the hardness thereof which comprises heating such a metal in an inert atmosphere in contact with only a refractory consisting essentially of  $\text{CaO}$ ,  $\text{ZrO}_2$  and  $\text{TiO}_2$ .

40 2. A process for fusing high-melting reactive metals of the class consisting of titanium and titanium-base alloys without significantly increasing the hardness thereof which consists in heating such a metal above its melting point while maintaining it in contact with only an inert atmosphere and a refractory body which consists essentially of 90% to 39%  $\text{CaO}$ , 7% to 27%  $\text{ZrO}_2$  and 3% to 24%  $\text{TiO}_2$ .

45 3. A process for fusing high-melting reactive metals of the class consisting of titanium and titanium-base alloys without significantly increasing the hardness thereof which comprises heating such a metal in an inert atmosphere and in a container formed essentially of 90% to 39%  $\text{CaO}$ , 7% to 37%  $\text{ZrO}_2$  and 3% to 24%  $\text{TiO}_2$ .

50 4. A process for fusing high-melting reactive metals of the class consisting of titanium and titanium-base al-

loys without significantly increasing the hardness thereof which comprises placing such a metal in a container having a composition, exclusive of impurities, of from 90% to 39% CaO, 7% to 37% ZrO<sub>2</sub> and 3% to 24% TiO<sub>2</sub>, and heating said metal in an inert atmosphere. 5

## References Cited in the file of this patent

UNITED STATES PATENTS  
2,205,854 Kroll June 25, 1940 10

2,402,516 Wainer June 18, 1946  
2,402,517 Wainer June 18, 1946  
2,452,532 Wainer Oct. 26, 1948  
2,541,140 Woodcock et al. Feb. 13, 1951  
5 2,678,887 Hathaway III May 18, 1954  
2,684,297 Urban July 20, 1954

## FOREIGN PATENTS

594,020 Great Britain Oct. 31, 1947  
659,475 Great Britain Oct. 24, 1951